

May 27, 1969

, 1965 P. E. SHICK 3,446,698  
METHOD OF IMPREGNATING AND DIGESTING CELLULOSIC MATERIALS  
IN A HORIZONTAL DIGESTOR  
Filed June 1, 1965



BY W. A. Schaich &  
Thomas A. Meelham  
ATTORNEYS

**1**

3,446,698

**METHOD OF IMPREGNATING AND DIGESTING CELLULOSIC MATERIALS IN A HORIZONTAL DIGESTOR**

Philip E. Shick, Toledo, Ohio, assignor to Owens-Illinois, Inc., a corporation of Ohio

Filed June 1, 1965, Ser. No. 460,371

Int. Cl. D21c 7/00

U.S. CL. 162—19

2 Claims

**ABSTRACT OF THE DISCLOSURE**

This invention relates to a process for continuously digesting wood chips wherein two connected treating zones are utilized. In the first zone, the wood chips are impregnated with a digesting liquor. Likewise, the first zone contains, in addition to the chips and the digested liquid, a non-condensed gas, said non-condensed gas generally keeping the temperature of said reaction zone such that effective impregnation of the chips with the digesting liquor is possible. Under impregnation, the chips are then passed to a second zone, the chips and digesting liquor are exposed to steam in such a fashion that the temperature is caused to rise to a point where digestion is effected. The atmosphere of the first zone essentially comprises a non-condensed gas, while the atmosphere of the second zone comprises essentially steam.

The present invention relates to a novel method and novel apparatus of utility in the manufacture of paper. Most particularly, the present invention relates to the manufacture of paper pulp by means of digestion of ligno cellulosic substances such as wood chips. More specifically, the present invention relates to such apparatus, methods, techniques and systems embodying features of novelty in a particular achievement of pressure above atmospheric in order to achieve efficient impregnation of the cellulose source, usually wood chips.

It has long been recognized that pressure impregnation of cellulose fiber-yielding substances results in improved yield as well as economy of pulping operations. The Pandia Division of Black-Clawson Company of Hamilton, Ohio, markets a line of pressure digesters featuring multiple reactors in series having internal pulp-moving screws and heat/pressure influencing components providing controlled and timed movement of the, for example, wood chips through the heat and pressure zone, thereby providing, it is alleged, improved impregnation and improved pulp production efficiency.

The present invention relates generally to pressure pulp digester units and particularly to such units of improved performance in terms of pulping efficiency, both as to yield and improved character of the ultimate pulp.

Pressure tube digesting reactor units marketed by the Pandia Division of Black-Clawson Company, can be modified to incorporate a valve between, for example, two vertically spaced horizontal tubes used for sequential movement of the wood chips and the ultimate pulp therethrough whereby difference in temperature and pressure conditions can be maintained for each section providing selective control of impregnation and control of pressure and temperature conditions in each zone in order to achieve a desirable and complete pulping. The use of these intermediate valves has proven expensive as to installation and operation. Additionally, operation has not

**2**

proven eminently smooth or satisfactory in the accomplishment of their designed ends.

Accordingly, it is an object of the present invention to provide improved apparatus and methods which obviate the necessity of employing special intermediate valves in sequential, zoned, pressure tube reactors for digestion of cellulose-producing substances, e.g., wood chips.

It is a particular object of the present invention to provide a system which in operation, both as to the apparatus and method, avoids the presence, in the resultant pulp, of chips having incompletely cooked centers.

It is still another object of the present invention to provide a pulping system which is capable of producing a pulp of considerably greater brightness than known heretofore.

It is a particular object of the present invention to provide a method and apparatus which together combine and cooperate to give an improved pulping system as compared to those known heretofore.

It is still another object of the present invention to provide a pulping system which, in terms of method and apparatus, is capable of facile control and operation and yet is marked by pulp of greater brightness and representing a more efficient system in toto.

It is yet another object of the present invention to provide a pulping system including method and apparatus which in operation provides improved impregnation of the cellulose source, e.g., the wood chip, such that the efficiency of pulping is markedly increased as to yield and as to quality of pulp produced.

The foregoing as well as other objects of the present invention will become apparent to those skilled in the art from the following detailed description taken in conjunction with the annexed sheet of drawings on which there is presented, for purposes of illustration, a single embodiment of the present invention.

In the drawings:

The figure is a partially schematic, partially sectional side elevation view of an array of pulping apparatus components shown in interrelated operative condition and thereby adapted to yield digested pulp ready for introduction into a refiner, a defibrator or the like.

In its simplest embodiment, the present invention contemplates the discovery that improved impregnation can be achieved by a method and apparatus which embodies features of construction and operation providing separate pressure zones in an otherwise unitary pressure digesting reactor tube system. By the expedient of selective location for the introduction of the impregnating high temperature steam and selective location for introduction of a noncondensable gas medium, an elevated pressure is achieved without accompanying elevated temperatures.

In a particular embodiment, the non-condensable gas is introduced, substantially contemporaneously with the wood chips, to a first horizontal reactor tube, defining a first zone, equipped with chip-transporting helical blades which propel the chips smoothly, uniformly and horizontally transversely therethrough to a connect conduit which in turn leads to a second horizontal reactor tube, defining a second zone, equipped with chip and/or transporting helical blades and said tube, defining a second zone, being furnished with a steam inlet arrangement for introducing, into contact with the now pressure-impregnated chips, high temperature steam. Preferably, digesting liquor or the chemical or semi-chemical type, e.g., sulphite, acid sulphite, bisulphite or sulphate type,

etc., is introduced into the first reactor tube about contemporaneously with the introduced wood chips and the introduced non-condensable gas, whereby the impregnation, rapid neutralization and initial pulping reactions take place under these conditions of high pressure but of low temperature.

An understanding of the present invention will be more apparent to those skilled in the art from the following more detailed discussion in which reference will be had to FIG. 1; which figure serves to illustrate both the method and apparatus of the present invention.

In the figure, a feed hopper 11 is situated vertically above and fluidly in connection with a tubular feeder 13 containing a rotatable helical blade 14 extending from shaft 14a. The hopper 11 connects with the feeder through a cylindrical vertical inlet opening 12. The feeder includes a converging wall section 15 fluidly connecting with an inlet pipe 18 which extends downwardly to connect with the first reactor tube 20 situated horizontally, as illustrated. The outlet end 21 of the tubular reactor 20 connects fluidly with a vertical transfer conduit 23 which connects with a tubular reactor tube 25 of the present invention, which is similar in construction to the reactor tube 20. The reactor tube 25 includes an inlet end 26 which connects with the vertical transfer pipe 23 at one end with a downwardly opening outlet pipe 27 which connects with a pocket type rotary discharger 28, as shown. Returning to inlet 18, conduit 30 connects therewith opposite the feed hopper outlet 16 and connects via line 31, control valve 32, line 33, pressure regulator 34, line 35 and valve 37, with a pressure cylinder 36 of nitrogen. Line 38 connects with line 30 via T 39 and leads to a pressure gauge 40.

The tubular reactor 20 has connected thereto a line 41 connecting with a pressure gauge 42 at the inlet end proximate inlet pipe 18. A temperature gauge 43 is located at the outlet end 21 of reactor tube 20. A similar temperature gauge 44 extends into the inlet end 26 of tubular reactor 25 proximate the vertical transfer pipe 23.

Conduit 45 leads into the tubular reactor 20 proximate the inlet pipe 18 and extends from the discharge side of a pump 46 mounted on base 47. Conduit 48 leads from a supply tank, 48a, of digesting liquor, via a metering pump, 48b, to the inlet end of centrifugal pump 46. Conduit 49 leads from the lower segment of reactor tube 20, as shown, to connect with conduit 48 leading to the liquor circulating pump 46. Conduit 50 exits into vertical transfer pipe 23 and serves for introduction of steam proceeding through valve 51. Conduit 50 is equipped with a pressure gauge 52.

The rotary discharger 28 includes a cylindrical shell 28a in which rotates a hollow central tube 28b having a central perforate wall 28c. The element 28b in rotation connects oppositely disposed tubular conduits 54 and 56; the latter of which connects with an air supply. The rotatable tube member 28b can also connect with the outlet 27 whereupon the steam pressure in the system will fill one half of the member 28b with a supply of digested pulp, as shown. Rotation of the tube 28b, a one-quarter turn, causes it to connect with outlet 54, whereupon a blast introduced through conduit 56 will push the pulp by means of the perforate plate 28c outwardly to a blow tank, for example. Continued rotation of the tube 28b causes a repetition of the just described exhaust procedure.

In operation, wood chips 61 of relatively uniform size are located in the hopper 11 from which they drop through the outlet 12 into the cylindrical feeder 13. Blades 14 rotating on shaft 14a pressure pack the chips (by reason of the converging wall section 15) into plugs which proceed through the outlet 16 onto the inlet pipe 18 from which the chips fall by gravity downwardly into the first tubular reactor 20. The formation of the plugs serves as a pressure seal against loss of pressure within the tube reactors 20 and 25. Rotating helical blade 20a propels the chips laterally to the outlet end 21. Contem-

poraneously with the introduction of the chips, a non-condensable gas, for example, nitrogen, is introduced through the conduit 30. Simultaneously, a liquor, capable of attacking the lignins and encrustations or binding components holding the wood cellulose fibers together, is introduced through conduit 45 into intimate contact with the chips being propelled along the reactor 20. From the outlet end, the wood chips, substantially separated from the liquor which exits through outlet line 49, pass downwardly through transfer pipe 23 into the lower tubular reactor 25 wherein they are propelled reversely to the left by helical blade 25a to pass downwardly out the outlet 27. As the chips drop through the transfer conduit 23, they are contacted by inlet steam entering through the line 50. The digested wood pulp or exhausted chips pass thence out outlet 27 into the pocket-type rotary discharger where they are discharged to a blow tank in conventional fashion. It is a feature of the present invention that the temperature within the tubular reactor 20 can be maintained at a substantially lower temperature, for example, approximately 15° to 30° less, than the temperature maintained within the tubular reactor 25. This is accomplished by reason of the introduction of the steam into the transfer conduit 23, rather than into the first reactor in accordance with conventional practice. Contemporaneously and also a controlling factor in the maintenance of the lesser temperature in the first tubular reactor is the provision for introduction of a non-condensable "padding" gas, as it were, such as nitrogen, through the inlet conduit 30 proximate the location at which the wood chips are introduced into the tubular conduit reactor tube 20. The introduction of the non-condensable gas creates a positive "padding" pressure of said gas, precluding or reducing passage of the inlet steam (entering through conduit 50) upward into the confines of the tubular reactor 20. By reason of the introduction of the non-condensable nitrogen and also by reason of the passage of the wood chips via the helical blade 20a in the tubular reactor 20 and the helical blade 25a in reactor 25, the steam is urged positively downwardly and then laterally to the left and is entrained with the liquor-impregnated wood chips.

An apparatus as described in FIG. 1 was operated in accordance with the present invention in order to determine the effect of the introduction of a non-condensable gas. Chips utilized in the series of experiments consisted primarily of oak wood having a typical analysis as follows:

|                | Percent |
|----------------|---------|
| 50 Lignin      | 25.2    |
| Alphacellulose | 45.7    |
| Hemicellulose  | 23.2    |

The chips had a specific gravity of 0.521 and a moisture content of 37.8%.

#### Example I

The apparatus as just described was operated wherein chips as described were introduced into a tubular reactor into which was introduced a digesting liquor having the following composition.

| Substance:                                          | Grams per liter<br>calculated as Na <sub>2</sub> O |
|-----------------------------------------------------|----------------------------------------------------|
| 65 NaHS                                             | 6.1                                                |
| Na <sub>2</sub> S <sub>2</sub> O <sub>3</sub>       | 11.8                                               |
| Na <sub>2</sub> SO <sub>3</sub>                     | 33.8                                               |
| Na <sub>2</sub> CO <sub>3</sub> +NaHCO <sub>3</sub> | 46.4                                               |

Table I below lists the conditions including the following: 70 the time of the run ranging from 0 to 29 minutes; the steam pressure reading of steam gauge 52; the pressure within the nitrogen supply tank in pounds per square inch gauge; the nitrogen pressure at the inlet to the digester inlet pipe 18 at gauge 40; the temperature in the top reactor tube as taken on temperature gauge 43; the tem-

perature in the bottom tube reactor 25 as recorded from temperature gauge 44; and the flow rate of the nitrogen in pound moles per minute.

T472-51. The brightness tests were conducted in accordance with TAPPI Standard Method T452 M-58 using Photovolt Corporation's Reflection Meter Model 610. As

TABLE 1

| Time<br>(min.) | Steam<br>pres.<br>(p.s.i.g.)<br>(ga. 52) <sup>1</sup> | Nitrogen<br>tank<br>pres.<br>(p.s.i.g.) | Nitrogen<br>pres.<br>at inlet<br>to digest<br>(ga. 40) <sup>1</sup> | Top<br>tube<br>temp.,<br>°F.<br>(ga. 43) <sup>1</sup> | Bottom<br>tube<br>temp.,<br>°F.<br>(ga. 44) <sup>1</sup> | Nitrogen<br>flow rate<br>in interval<br>calculated<br>lb. mole/min. |
|----------------|-------------------------------------------------------|-----------------------------------------|---------------------------------------------------------------------|-------------------------------------------------------|----------------------------------------------------------|---------------------------------------------------------------------|
| 0.....         | 155                                                   | 1,500                                   | 178                                                                 | 350                                                   | 350                                                      | -----                                                               |
| 5.....         | 160                                                   | 1,200                                   | 185                                                                 | 340                                                   | 350                                                      | 0.0108                                                              |
| 7.....         | 155                                                   | 1,080                                   | 180                                                                 | 330                                                   | 350                                                      | 0.0108                                                              |
| 10.....        | 155                                                   | 950                                     | 175                                                                 | 325                                                   | 349                                                      | 0.0078                                                              |
| 12.....        | 150                                                   | 850                                     | 176                                                                 | 320                                                   | 346                                                      | 0.0090                                                              |
| 14.....        | 150                                                   | 780                                     | 170                                                                 | 315                                                   | 344                                                      | 0.0063                                                              |
| 16.....        | 145                                                   | 670                                     | 187                                                                 | 318                                                   | 344                                                      | 0.0099                                                              |
| 18.....        | 150                                                   | 590                                     | 180                                                                 | 324                                                   | 346                                                      | 0.0072                                                              |
| 20.....        | 150                                                   | 540                                     | 178                                                                 | 323                                                   | 347                                                      | 0.0045                                                              |
| 22.....        | 150                                                   | 450                                     | 175                                                                 | 327                                                   | 347                                                      | 0.0054                                                              |
| 25.....        | 150                                                   | 390                                     | 170                                                                 | 326                                                   | 346                                                      | 0.0054                                                              |
| 27.....        | 148                                                   | 350                                     | 188                                                                 | 324                                                   | 346                                                      | 0.0036                                                              |
| 29.....        | 150                                                   | 200                                     | 188                                                                 | 325                                                   | 346                                                      | 0.0135                                                              |

<sup>1</sup> Refers to gauge illustrated in drawings. The flow rate of the chips, measuring about  $\frac{1}{2}$  inch in diameter on an average, was adjusted to 444 grams per minute of O.D. (oven dry) wood. The flow rate was controlled so that the residence time of any given chip within the digester reactor tubes was about 14 minutes in total. The liquor flow rate was controlled to measure 407 cubic centimeters per minute. The resulting pulp was blown into a flat bottom wash screen for a period of 4 minutes. Thereafter, the timed sample was washed for 20 minutes with hot water and then 10 minutes with cold water. The pulp was then put through a disc refiner manufactured by Sprout Waldron in a flow of water achieving a complete washing while defibering the chips. The resulting pulp was thickened on an 80 mesh screen and allowed to drain for approximately 15 minutes and then centrifuged to approximately 20% consistency. This spun dried pulp was then crumbled and five 200 gram samples were taken for moisture determination. The remaining pulp was placed in a polyethylene bag which was sealed airtight to guard against any change in moisture content. The 200 gram samples were placed in tin cans and weighed within 0.1 gram. The samples were oven dried at 105-110° overnight.

### Example II

Using the same apparatus, a duplicate amount of chips and a duplicate amount of liquor as in Example I, another run was carried out differing only in that no non-condensable nitrogen was introduced into the system. It was noted during this run that the temperatures indicated on gauge 43 and 44 (upper and lower reactor tubes, respectively) were approximately the same, e.g., 350° F.

The pulps produced and collected in accordance with Examples I and II were formed into paper sheets which were subjected to a "Mullen" test, a tear test and a ring crush and the results summarized in Table 2.

TABLE 2

|                                              | Example I | "Control" |
|----------------------------------------------|-----------|-----------|
| Mullen (p.s.i.).....                         | 31        | 36        |
| Tear (gram/16 sheets).....                   | 55        | 52        |
| Ring Crush (lbs./ $\frac{1}{4}$ " x 6")..... | 57        | 55        |
| GE photovolt brightness (percent).....       | 19.5      | 11.5      |
| Yield <sup>1</sup> .....                     | 67.6      | -----     |

<sup>1</sup> Yield is obtained by dividing the oven dried pulp produced during the 4 minute run, divided by the total of oven dried wood fed to the digester during the same interval.

The Mullen Bursting Strength Test was determined using a B. F. Perkins' Mullen Tester ranging from 0-120 p.s.i. in accordance with TAPPI Standard Method T403 TS-63.

30 can be seen, the brightness of the paper was higher by a sizeable factor, e.g., 8 points, (19.5-11.5) which approaches a 100% improvement.

### Example III

35 In another set of runs, a liquor having the following analysis was utilized.

| Substance:                                          | Grams per liter<br>calculated as Na <sub>2</sub> O |
|-----------------------------------------------------|----------------------------------------------------|
| NaHS                                                | 5.2                                                |
| Na <sub>2</sub> S <sub>2</sub> O <sub>3</sub>       | 13.0                                               |
| Na <sub>2</sub> SO <sub>3</sub>                     | 32.2                                               |
| Na <sub>2</sub> CO <sub>3</sub> +NaHCO <sub>3</sub> | 50.3                                               |

45 In this run, the same chips as before were utilized but at a flow rate of 434 grams per minute on the basis of oven dried wood, while the liquor flow rate was set at 391 cubic centimeters per minute.

Table 3 below lists the duration of the run in minutes (33) as well as time increments during which the steam pressure was taken on pressure gauge 52 together with the nitrogen tank pressure in p.s.i.g., the nitrogen pressure at the inlet to the digester tube 18 taken on pressure gauge 40 together with the temperature taken on gauge 43, the temperature taken on gauge 44, the digester pressure taken on gauge 42 and the nitrogen flow rate during the incremental time elements in pound moles per minute.

TABLE 3

| Time<br>(min.) | Steam<br>pres.<br>(p.s.i.g.)<br>(ga. 52) <sup>1</sup> | Nitrogen<br>Tank<br>pres.<br>(p.s.i.g.) | Nitrogen<br>pres.<br>at inlet<br>to digest<br>(p.s.i.g.)<br>(ga. 40) <sup>1</sup> | Top<br>tube<br>temp.,<br>°F.<br>(ga. 43) <sup>1</sup> | Bottom<br>tube<br>temp.,<br>°F.<br>(ga. 44) <sup>1</sup> | Digester<br>pres.<br>(p.s.i.g.)<br>(ga. 42) <sup>1</sup> | Nitrogen<br>flow rate<br>in interval<br>calculated,<br>lb. mole/min. |
|----------------|-------------------------------------------------------|-----------------------------------------|-----------------------------------------------------------------------------------|-------------------------------------------------------|----------------------------------------------------------|----------------------------------------------------------|----------------------------------------------------------------------|
| 0.....         | 160                                                   | 2,275                                   | 165                                                                               | 360                                                   | 360                                                      | 165                                                      | -----                                                                |
| 3.....         | 160                                                   | 1,960                                   | 165                                                                               | 340                                                   | 360                                                      | 170                                                      | 0.0189                                                               |
| 10.....        | 160                                                   | 1,620                                   | 165                                                                               | 320                                                   | 346                                                      | 170                                                      | 0.0087                                                               |
| 13.....        | 160                                                   | 1,580                                   | 170                                                                               | 348                                                   | 361                                                      | 170                                                      | 0.0024                                                               |
| 17.....        | 165                                                   | 1,400                                   | 170                                                                               | 335                                                   | 356                                                      | 170                                                      | 0.0081                                                               |
| 19.....        | 165                                                   | 1,300                                   | 170                                                                               | 330                                                   | 356                                                      | 175                                                      | 0.0090                                                               |
| 21.....        | 165                                                   | 1,210                                   | 175                                                                               | 330                                                   | 356                                                      | 170                                                      | 0.0171                                                               |
| 22.....        | 165                                                   | 1,150                                   | 170                                                                               | 330                                                   | 356                                                      | 170                                                      | 0.0054                                                               |
| 25.....        | 165                                                   | 1,090                                   | 170                                                                               | 330                                                   | 354                                                      | 167                                                      | 0.0054                                                               |
| 27.....        | 163                                                   | 990                                     | 170                                                                               | 330                                                   | 355                                                      | 167                                                      | 0.0090                                                               |
| 29.....        | 165                                                   | 900                                     | 170                                                                               | 335                                                   | 356                                                      | 170                                                      | 0.0081                                                               |
| 31.....        | 165                                                   | 820                                     | 170                                                                               | 335                                                   | 357                                                      | 170                                                      | 0.0072                                                               |
| 33.....        | 165                                                   | 750                                     | 170                                                                               | 335                                                   | 355                                                      | 170                                                      | 0.0063                                                               |

<sup>1</sup> Refers to gauge illustrated in drawings.

The tear resistance was determined on a standard Elmer-dorf Tearing Tester in accordance with TAPPI Standard Method T414 M-49. The ring crush of the samples was determined in accordance with TAPPI Standard Method

### Example IV

A run identical to that of Example III was conducted 55 over the same time interval and having the same read-

ings in terms of pressures, rates, etc., excepting that no nitrogen was introduced into the reactor tube digester. The same chip flow rate was maintained as well as the liquor flow rate. The yield in each case was calculated as described hereinabove with Examples I and II. The results of tests performed on paper formed from the two sets of pulp are summarized in Table 4 below:

TABLE 4

|                                         | Example III | "Control"<br>Example IV |
|-----------------------------------------|-------------|-------------------------|
| Mullen (p.s.i.)                         | 31          | 28                      |
| Tear (gram/16 sheets)                   | 57          | 53                      |
| Ring Crush (lbs./ $\frac{1}{2}''$ x 6") | 58          | 52                      |
| GE photovolt brightness (percent)       | 18.5        | 11.5                    |
| Yield <sup>1</sup>                      | 66          | 63.9                    |

<sup>1</sup> Yield is obtained by dividing the oven dried pulp produced during the 4 minute run, divided by the total of oven dried wood fed to the digester during the same interval.

It may be noted from Table 3 that the top tube temperatures ran between 20 and 26° F. cooler than the temperature in the bottom tube, demonstrating that paper of as good or better properties could be achieved with less rigorous pulping temperatures although at the same pressure.

The reason for the increased brightness when utilizing the system of the present invention, wherein a non-condensable gas such as nitrogen is introduced into the primary digester reactor tube, is not known.

Applicant has thus found that digestion of the cellulose-yielding wood chip is improved where the first stage of the digestion is accomplished at a lower temperature provided by reason of the "padding" atmosphere produced by introducing a non-condensable gas, such as nitrogen, contemporaneous with the introduced wood chips and contemporaneous with the introduction of the cooking liquor.

My invention is not to be considered limited to the production of pulp and/or fiber from wood chip and wood waste but, of course, is applicable to the production of pulp and fiber, for example, from any cellulosic starting material such as flax, wheat and other straws, grasses, bagasse, linters, etc.

While only nitrogen has been utilized in the aforesaid examples, it will be appreciated that air under certain circumstances, as well as other gases, may be substituted in whole or in part; their choice being based upon a proper consideration of the digesting liquor, the nature of the cellulose-contributing substance, etc.; care being taken to select a gas which is relatively, e.g., substantially, non-condensable. A substantially non-condensable gas is one which tends not to condense within the digester tube reactor. Stated conversely, a relatively non-condensable gas is one which tends to remain a gas within the tubular reactor and thus available to fulfill its function of precluding entry of steam into the inlet region of the tubular reactor. Thus, it will be appreciated that oxygen will serve as a suitable relatively non-condensable gas with certain pulp digesting cooks. Ammonia (NH<sub>3</sub>) is a suitable non-condensable gas in alkaline cooks while gases such as sulfur dioxide (SO<sub>2</sub>) and carbon dioxide (CO<sub>2</sub>) are suit-

able non-condensable gases for acid cooks. The so-called "combustion gases" are also candidate non-condensable gases, assuming appropriate care in the matching of "combustion gas" component and the nature and character of the particular cook involved.

Having in mind (1) overall efficiency of pulping, regardless of the character of the cook (alkaline or acid), (2) the optimum in properties of the ultimate sheet and (3) the chemical inertness of nitrogen; it is most preferred to use nitrogen as the non-condensable gas in the digestion of cellulosic substances in accordance with the present invention.

I claim:

1. The method of converting lignocellulosic material into pulp which comprises:

introducing said material into a first substantially horizontal chamber together with a chemical adapted to digest the binding lignin ingredients and encrusting substances holding cellulose fibers together, introducing a non-condensable gas into said first chamber, said material being resident in said first chamber for a period of time sufficient to effect impregnation, passing said material from said first chamber directly into a second substantially horizontal chamber, introducing steam into said material and said second chamber adjacent the point of introduction of said material into said second chamber to thereby raise the temperature in said second chamber to a level greater than the temperature in said first chamber, controlling the pressure of said non-condensable gas in the first chamber so that said first chamber is maintained at a higher pressure than said second chamber thereby substantially prohibiting the migration of the steam from said second chamber to said first chamber,

passing said material and steam through said second chamber at said greater temperature whereby digestion proceeds,

said material being resident in said second chamber for a period of time sufficient to effect digestion, and discharging said material.

2. The method as claimed in claim 1 wherein said non-condensable gas is nitrogen.

#### References Cited

##### UNITED STATES PATENTS

|           |         |                     |           |
|-----------|---------|---------------------|-----------|
| 2,858,213 | 10/1958 | Durant et al. ----- | 162—237 X |
| 2,963,086 | 12/1960 | Green -----         | 162—237   |
| 3,294,625 | 12/1966 | Gessner -----       | 162—68    |
| 3,308,011 | 3/1967  | Ross -----          | 162—68    |

S. LEON BASHORE, Primary Examiner.

R. D. BAJEFSKY, Assistant Examiner.

U.S. Cl. X.R.

162—18, 68, 237